# EUROPEAN PATENT APPLICATION

(11) **EP 1 136 579 A1**
(43) Date of publication of application: **26.09.2001**
(21) Application number: 01302434.4
(22) Date of filing: 16.03.2001
(51) Int. Cl.: C22C 38/00

(54) **Ultra low carbon boron steels (ULCB) for applications requiring extreme drawability and/or cold formability**

(30) Priority: 22.03.2000 GB 0006798
(71) Applicant: Corus UK Limited, London W1V 2BS (GB)
(72) Inventor: Bell, Andrew, c/o Corus Research Develop.&Techn., Rotherham, South Yorkshire, S60 3AR (GB); Hallgarth, J K, c/o Corus Research Develop.&Techn., Rotherham, South Yorkshire, S60 3AR (GB)
(74) Representative: Townsend, Victoria Jayne

(57) **Abstract**

An ultra-low carbon boron steel comprises by weigh per cent: not more than 0.01% C, not more than 0.01% Si, not more than 0.25% Mn, not more than 0.05% Al, approximately 0.0025% to 0.0035% N and between 0.0020% and 0.0050% B, the remainder being iron and incidental elements and impurities, wherein the weight ratio of B:N is between about 0.68 and 0.90. The steel can be continuously cast and processed for applications requiring extreme drawability and cold formability.

## Description

The present invention relates to a continuously cast, boron treated ultra-low carbon steel (ULCB) for use in applications where:-
(i) extreme drawability and / or
(ii) cold formability is required.

More specifically, the invention relates to a steel having an ultra-low carbon content and a boron addition which has drawability and cold formability comparable to or better than that of conventional ingot cast rimming steels, other continuously cast rimming steel substitutes and aluminium treated low carbon cold heading steels. The present invention also relates to a process for producing such continuously cast boron treated ultra-low carbon steel as as-cast blooms, hot rolled billet, bar and rod.

There is a current trend within the steelmaking industry to move away from the traditional method of ingot casting and towards the newer, more efficient continuous casting method. Unfortunately, certain types of steel do not lend themselves to the continuous casting method and replacement steels have had to be developed. One of the steel types that is not suited to continuous casting, namely rimming steel, is utilised in the drawing of fine wires, e.g. for use in glass reinforcing mesh, and the drawing of larger wire diameters for subsequent use in cold heading operations to form components such as rivets. Rimming steels possess excellent drawability due to the presence of a virtually pure iron rim around the surface of the rod. This rim work hardens at a lower rate than the body of the steel during drawing and is very forgiving of any surface defects. The rim is developed by controlling the effervescence of CO gas during the solidification process. Unfortunately, the continuous casting process does not facilitate control of the gas evolution during solidification and a virtually pure iron rim cannot be formed by this method. Several rimming substitute steels have been developed for use in applications such as these, but as yet, none have possessed the drawability or cold formability of ingot cast rimming steels.

An objective of the present invention is to provide billet feedstock and a hot rolled steel bar or wire rod of a chemical composition giving lower tensile strength, higher ductility and a lower work hardening rate resulting in enhanced drawability and cold formability compared with the levels usually found in ingot cast rimming steels and other rimming steel substitutes. The resulting drawn wire products have a variety of applications. Large diameter drawn wires, for instance, can be cold headed to form rivets, whilst smaller drawn wires sizes (0.51,0.66 and 0.71mm) find application in glass reinforcement mesh.

In accordance with the present invention there is provided a boron treated ultra-low carbon boron steel comprising by weight per cent: not more than 0.01 % C, not more than 0.01% Si, not more than 0.25% Mn, not more than 0.05% Al, approximately 0.0025% to 0.0035% N and between 0.0020% and 0.0050% B, the remainder being iron and incidental elements and impurities, wherein the weight ratio of B:N is between about 0.68 and 0.90.

Preferably the quantity of carbon is not more than about 0.007%.

Preferably the weight ratio of B:N is about 0.79. The free nitrogen available in the processed steel is preferably less than 0.001 % and preferably less than about 0.0007%.

In a second aspect, the invention is a steel billet, hot rolled bar or rod or cold drawn wire, the steel comprising by weight per cent: not more than 0.01 % C, not more than 0.01% Si, not more than 0.25% Mn, not more than 0.05% Al, approximately 0.0025% to 0.0035% N and between 0.0020% and 0.0050% B, the remainder being iron and incidental elements and impurities, wherein the weight ratio of B:N is between about 0.68 and 0.90.

In a third aspect, the invention is a method for manufacturing a rod or wire comprising the steps of;
continuously casting a steel having a composition by weight per cent of: not more than 0.01% C, not more than 0.01% Si, not more than 0.25% Mn, not more than 0.05% Al, approximately 0.0025% to 0.0035% N and between 0.0020% and 0.0050% B, the remainder being iron and incidental elements and impurities, wherein the weight ratio of B:N is between about 0.68 and 0.90;
producing the steel in the form of a billet suitable for further processing by hot rolling;
rolling the billet into a bar or rod at temperatures between 1100 and 830°C;
cooling at a rate sufficiently low to allow interstitial carbon to precipitate from solution;
drawing the rod to the desired wire diameter; and optionally
annealing the wire at a temperature suitable to develop the desired tensile strength and ductility in the wire product.

Ingot cast rimming steels have conventionally been used for extreme drawability applications. The inventors propose compositions of the present invention as continuously castable alternative steels for these purposes with comparable and in some cases superior properties to rimming ingot cast steels in these applications.

Figure 1 shows the work hardening curve for ULCB steel and ingot cast rimming steel (R06).

Figure 2 shows the ageing response of the ULCB and ingot cast rimming steel (R06) final wire.

Figure 3 shows the annealing response of the ULCB and ingot cast rimming steel (R06) final wire.

Figure 4 shows the tensile properties of 5.5mm ULCB, ELC (Corus™ grade) and SAE 1005-AL rimming substitute steel rod.

Steel materials according to the present invention may be used in the production of wires destined for use in two distinct and separate applications, namely:-
(i) applications requiring extreme drawability, e.g. production of fine wire feedstock (0.71-0.51mm diameter) for the manufacture of mesh for glass reinforcement mesh.
(ii) applications requiring a high degree of cold formability, e.g. production of larger diameter wire feedstock for the manufacture of rivets via a cold heading operation.

The requirements of the present invention will be fully described with reference to the individual applications, however, the examples do not restrict the present invention.

### (i) ULCB Wire Rod for Extreme Drawability Applications

The following describes one suitable process route to obtain a wire for use in glass reinforcement made from the novel composition to which the present invention relates.

Steels of the previously described composition ranges are continuously cast into bloom and hot rolled to billet and then to 5.5 mm rod at temperatures between 1100 and 830°C using a continuous rod mill fitted with a Stelmor™ controlled cooling conveyor. The conveyor fan settings are kept relatively low so that the cooling rate on the conveyor is sufficiently slow to allow interstitial carbon to precipitate from solution, thus minimising any contribution to tensile strength in the end product.

The 5.5mm rod is descaled and drawn to 1.51mm using calcium soap then drawn to 0.51mm using sodium soap. The 0.51mm final wire may then be subsequently annealed at approximately 600-620°C to develop the required tensile strength and ductility in the wire end product.

The following gives the composition and mechanical properties of the rod and wire at the various stages of processing along with comparable data for an ingot cast rimming steel.

The product analyses of the rod and wire samples are shown in Table 1 as compared to an ingot cast rimming steel rod.

**TABLE 1**

| Material | Composition (wt %) | | | | | | | | |
|---|---|---|---|---|---|---|---|---|---|
| | C | Si | Mn | P | S | Al | B | O | N |
| ULCB Rod | 0.006 | <0.01 | 0.14 | 0.007 | 0.006 | 0.026 | 0.0023 | 0.0029 | 0.0033 |
| Ingot Cast Rimming Steel Rod | 0.021 | <0.01 | 0.22 | 0.011 | 0.009 | <0.005 | <0.0005 | 0.0300 | 0.0017 |
| Mo and Sn <0.005% and Cu <0.02%. | | | | | | | | | |

### Tensile Properties 5.5mm Rod

The tensile properties of the ULCB and ingot cast rimming steel rod samples are summarised in Table 2:-

**TABLE 2**

| Sample | Average TS (N/mm²) | Average R of A (%) |
|---|---|---|
| ULCB Rod | 314 | 92 |
| Ingot Cast Rimming Steel Rod | 342 | 81 |

### Microstructure

The microstructure of the ULCB rod consists almost entirely of ferrite grains (99.8 vol.%) with a very small amount of grain boundary/filamental carbide (0.2 vol.%).
The mean lineal intercept ferrite grain size are given in Table 3:-

**TABLE 3**

| Sample | MLI Ferrite Grain Size | |
|---|---|---|
| | (mm^{-1/2)} | (*µ*m) |
| ULCB Rod | 6.1 | 27 |
| Ingot Cast Rimming Steel Rod | 8.1 | 15 |

### Mechanical Properties of As-Drawn 1.51 mm wire

The mechanical properties of the as-drawn 1.51mm intermediate wire are given in Table 4. The 1.51mm intermediate wire was naturally aged at room temperature for up to 50 days. The change in tensile, torsion and reverse bend properties were followed throughout the ageing process. The changes in tensile properties are also given in Table 4 along with the changes in torsional and reverse bend properties.

**TABLE 4**

| Sample | | TS (N/mm²) | | R of A (%) | | Bend Ductility (No. of Bends) | | Torsional Ductility 100 d (Twists to Failure) | |
|---|---|---|---|---|---|---|---|---|---|
| | | Ave | Range | Ave | Range | Ave | Range | Ave | Range |
| ULCB | As-Drawn | 699 | 699 | 81 | 80-82 | 24 | 22-25 | 42 | 42 |
| | Aged 1 day | 686 | 680-691 | 76 | 76 | 24 | 23-25 | 42 | 42-43 |
| | Aged 5 days | 679 | 678-680 | 77 | 76-77 | 24 | 23-25 | 41 | 40-41 |
| | Aged 11 days | 716 | 707-724 | 77 | 77 | 24 | 23-25 | 42 | 42 |
| | Aged 20 days | 685 | 680-689 | 77 | 76-77 | 24 | 23-25 | 41 | 40-42 |
| | Aged 50 days | 701 | 688-714 | 77 | 76-78 | 25 | 24-26 | 41 | 41 |

A summary of all the observed properties is given below.
(a) Tensile Strength:-
   The tensile strength of the 1.51 mm intermediate wire changes by no more than 37 N/mm² over the 50 day ageing period.
(b) Tensile Ductility:-
   Following an initial drop, the tensile ductility (% R of A) of the 1.51 mm intermediate wire remains almost constant throughout the 50 day ageing period.
(c) Reverse Bend Ductility/Torsional Ductility:-
   There was virtually no change in either reverse bend ductility or torsional ductility of the 1.51 mm intermediate wire throughout the 50 day ageing period.

### Mechanical Properties of As-Drawn 0.51mm wire

The work hardening response of ULCB and ingot cast rimming steels during the drawing from 5.5mm rod to 0.51mm wire is represented graphically in Figure 1.

The mechanical properties of the as-drawn 0.51mm ULCB final wire are given in Table 5 along with comparable data for as-drawn 0.51mm ingot cast rimming steel wire.

**TABLE 5**

| Sample | | TS (N/mm²) | | R of A (%) | | Bend Ductility (No of Bends) | | Torsional Ductility 200 d (Twists to Failure) | |
|---|---|---|---|---|---|---|---|---|---|
| | | Ave | Range | Ave | Range | Ave | Range | Ave | Range |
| ULCB | As-Drawn | 1070 | 1065-1075 | 77 | 75-78 | 14 | 14-15 | 64 | 58-72 |
| | Aged 3 days | 1037 | 1034-1039 | 74 | 72-75 | 13 | 12-14 | 63 | 63-64 |
| | Aged 5 days | 1039 | 1039 | 77 | 75-78 | 13 | 13-14 | 62 | 58-63 |
| | Aged 12 days | 1039 | 1034-1044 | 75 | 75 | 14 | 14 | 6 | 58-77 |
| | Aged 20 days | 1054 | 1054 | 74 | 72-75 | 13 | 13-14 | 68 | 64-70 |
| | Aged 52 days | 1049 | 1044-1054 | 78 | 788 | 14 | 13-15 | 71 | 65-78 |
| Ingot Cast Rimming Steel | As-drawn | 1273 | 1268-1278 | 59 | 59 | 9 | 9 | 57 | 54-63 |
| | Aged 1 day | 1278 | 1268-1288 | 59 | 59 | 10 | 9-11 | 45 | 41-51 |
| | Aged 6 days | 1322 | 1317-1327 | 59 | 59 | 11 | 11 | 64 | 58-64 |
| | Aged 11 days | 1287 | 1277-1297 | 59 | 59 | 10 | 9-11 | 47 | 39-54 |
| | Aged 50 days | 1251 | 1246-1256 | 61 | 59-63 | 10 | 9-12 | 50 | 48-55 |

The 0.51mm wire was naturally aged at room temperature for up to 50 days. The change in tensile, torsion and reverse bend properties were followed throughout the ageing process. The changes in tensile properties are given in Table 5 and presented graphically in Figure 2. The changes in torsional and reverse bend properties are also given in Table 5.

A summary of the observed properties is given below.
(a) Tensile Strength:-
   The tensile strength of the ULCB 0.51mm final wire varies by no more than 31N/mm² over the 50 day ageing period, compared with a variation of 71N/mm² in the ingot cast rimming steel.
(b) Tensile Ductility:-
   The tensile ductility of both the 0.51mm ULCB and ingot cast rimming steel final wire remains relatively unchanged during the 50 day ageing period. At ∼76%, the level of tensile ductility in the ULCB steel is higher than the 59% found in the ingot cast rimming steel.
(c) Reverse Bend
   There was virtually no change in the reverse bend ductility of either the ULCB or the ingot cast rimming steel wire throughout the 50 day ageing period.
(d) Torsional Ductility:-
   The torsional ductility of the 0.51mm ULCB final wire showed a slight rise during the 50 day ageing period. The torsional ductility of the 0.51mm ingot cast rimming steel final wire exhibited a large degree of scatter over the 50 day ageing period.

### Mechanical Properties of Annealed 0.51mm wire

The tensile properties of laboratory annealed 0.51mm ULCB final wire are given in Table 6 along with comparable data for as-drawn 0.51mm ingot cast rimming steel wire and are presented graphically in Figure 3.

**TABLE 6**

| Steel | Annealing Temperature (°C) | Tensile Strength (N/mm²) | | R of A (%) | |
|---|---|---|---|---|---|
| | | Average | Range | Average | Range |
| ULCB | 550 | 387 | 382-392 | 91 | 91 |
| | 575 | 392 | 392 | 90 | 89-90 |
| | 600 | 353 | 353 | 92 | 92 |
| | 625 | 314 | 312-315 | 93 | 92-93 |
| | 700 | 274 | 251-297 | 86 | 85-87 |
| | 800 | 245 | 243-248 | 85 | 82-87 |
| Rimming Steel | 550 | 319 | 317-320 | 85 | 83-86 |
| | 575 | 312 | 311-312 | 84 | 83-85 |
| | 600 | 292 | 291-293 | 88 | 87-88 |
| | 625 | 313 | 308-317 | 85 | 81-88 |
| | 700 | 260 | 256-264 | 80 | 78-82 |
| | 800 | 190 | 181-198 | 84 | 82-85 |

### (ii) ULCB Wire Rod for Applications Requiring a High Degree of Cold Formability

The following describes one suitable process route to obtain a wire for use in applications requiring a high degree of cold formability (such as the production of rivets via a cold heading operation) made from the novel composition to which the present invention relates.

Steels of the previously described composition ranges are continuously cast into bloom and hot rolled to billet, rod and then to bar or rod at temperatures between 1100 and 830°C using a continuous rod mill fitted with a Stelmor™ controlled cooling conveyor. The conveyor fan settings are kept relatively low so that the cooling rate on the conveyor is sufficiently slow to allow interstitial carbon to precipitate from solution, thus minimising any contribution to tensile strength in the wire product.

The following gives the composition and mechanical properties of 5.5mm ULCB rod along with comparable data for other continuously cast cold heading grades.

Typical product analyses of ULCB, ELC (Corus grade) and SAE 1005-AL steels are shown in Table 7.

**TABLE 7**

| Material | | Composition (wt %) | | | | | | | |
|---|---|---|---|---|---|---|---|---|---|
| | | C | Si | Mn | P | S | Al | N | B |
| ULCB | Typical | 0.006 | 0.006 | 0.20 | 0.004 | 0.006 | 0.030 | 0.003 | 0.0035 |
| | Min | - | - | 0.15 | - | - | 0.020 | - | 0.0020 |
| | Max | 0.010 | 0.010 | 0.25 | 0.015 | 0.015 | 0.050 | 0.005 | 0.0050 |
| ELC (Corus Grade) | Typical | 0.010 | 0.010 | 0.20 | 0.007 | 0.010 | 0.030 | 0.003 | |
| | Min | - | - | 0.15 | - | - | 0.020 | - | - |
| | Max | 0.030 | 0.020 | 0.25 | 0.025 | 0.025 | 0.050 | 0.007 | - |
| SAE 1005-AL | Typical | 0.040 | 0.010 | 0.25 | 0.015 | 0.018 | 0.035 | 0.004 | - |
| | Min | - | - | 0.20 | - | - | 0.020 | - | - |
| | Max | 0.060 | 0.050 | 0.40 | 0.035 | 0.035 | 0.050 | 0.007 | - |

Typical tensile properties of 5.5mm ULCB, ELC and SAE 1005-AL steel rod are summarised in Table 8 and represented graphically in Figure 4:-

**TABLE 8**

| Steel | Typical Mechanical Properties | |
|---|---|---|
| | Tensile Strength (N/mm²) | Tensile Reduction of Area (%) |
| ULCB | 280-320 | 90-95 |
| ELC | 310-350 | 83-88 |
| SAE 1005-AL | 335-375 | 75-80 |

The true stress-strain relationship for low carbon steels can be represented by the following equation:-${\text{σ = A.∈}}^{\text{n}}$

The corresponding values for the ULCB and SAE 1005-AL steels are given in Table 9:-

**TABLE 9**

| Steel Type | Values | |
|---|---|---|
| | A | n |
| ULCB | 533.0 | 0.214 |
| SAE 1005-AL | 635.5 | 0.244 |

The additional drawability of ULCB enables increased reductions in diameter without the requirement of an intermediate annealing operation prior to the cold heading operation. For example, cold heading can be performed on direct drawn

ULCB as compared with inter-annealed SAE 1005-AL. In addition, ULCB may also enable the production of more complex components without the risk of cracking.

The foregoing describes examples of a suitable manufacturing process and properties of just some compositions according to the present invention and is not intended to be limiting of the true scope of the invention as claimed in the appended claims.

## Claims

1. An ultra-low carbon boron steel comprising by weigh per cent:
not more than 0.01% C, not more than 0.01% Si, not more than 0.25% Mn, not more than 0.05% Al, approximately 0.0025% to 0.0035% N and between 0.0020% and 0.0050% B, the remainder being iron and incidental elements and impurities, wherein the weight ratio of B:N is between about 0.68 and 0.90.

2. An ultra-low carbon boron steel as,claimed in claim 1 wherein the quantity of carbon is not more than about 0.007%.

3. An ultra-low carbon boron steel as claimed in claim 2 wherein the C content is between about 0.004% and 0.005%.

4. An ultra-low carbon boron steel as claimed in any preceding claim wherein the weight ratio of B:N is between 0.68 and 0.90.

5. An ultra low carbon boron steel as claimed in claim 4 wherein the B:N ratio is about 0.79.

6. An ultra-low carbon boron steel as claimed in any preceding claim wherein the free nitrogen available in the processed steel is less than 0.001%.

7. An ultra low carbon boron steel as claimed in claim 8 wherein the free nitrogen available in the processed steel is less than 0.0007%.

8. A billet, bar, rod or wire comprising an ultra low carbon boron steel as claimed in any preceding claim.

9. A method for manufacturing a wire comprising the steps of;
continuously casting an ultra low carbon steel of the composition as claimed in any one of claims 1 to 7;
rolling the cast steel into a billet then to rod at a temperature of between about 1100 and 830°C;
cooling at a rate sufficiently low to allow interstitial carbon to precipitate from solution;
drawing the cooled rod to the desired wire diameter; and optionally
annealing the wire at a temperature suitable to develop the desired tensile strength and ductility in the wire product.

10. A method for providing a cold-headed metal article comprising the steps of:
continuously casting an ultra-low carbon steel of the compositions as claimed in any one of claims 1 to 7;
rolling the cast steel into a billet then to bar or rod at a temperature of between about 1100 and 830°C;
cooling at a rate sufficiently low to allow interstitial carbon to precipitate from solution;
drawing the cooled bar/rod to a desired wire diameter;
selecting a portion of the wire for the cold-headed product; and
cold heading the selected portion to form the product.

11. An ultra low carbon boron steel substantially as described herein.

12. A wire comprising ultra low carbon boron steel substantially as described herein.

13. A cold headed metal article comprising an ultra-low carbon boron steel substantially as described herein.

14. A method for manufacturing a wire substantially as described herein.

15. A method for manufacturing a cold-headed metal article substantially as described herein.
